

# UNITED STATES PATENT OFFICE.

ALADAR PACZ, OF CLEVELAND, OHIO, ASSIGNOR TO GENERAL ELECTRIC COMPANY, A CORPORATION OF NEW YORK.

## METHOD OF PRODUCING ALLOYS.

1,402,088.

Specification of Letters Patent. Patented Jan. 3, 1922.

No Drawing.

Application filed April 5, 1917. Serial No. 159,926.

To all whom it may concern:

Be it known that I, ALADAR PACZ, a citizen of the United States, residing at Cleveland, in the county of Cuyahoga and State 5 of Ohio, have invented a new and useful Method of Producing Alloys, of which the following is a specification.

My invention relates to the production of alloys and more particularly to the production of steel alloys containing tungsten, molybdenum, vanadium, chromium and other metals which serve to improve the properties of the steel for special purposes, tools, armor-plate, etc. The object of my invention is to produce an alloy having a much more uniform and intimate combination of the constituent metals than any heretofore produced.

According to my invention I mix very 20 intimately with the alloy metals a compound or mixture of compounds which is acid with respect to the oxides of the constituent alloy metals. That is to say the compounds are such as will unite with such oxides of 25 the alloy metals as may be present when these metals are fused together. It is generally more feasible to intimately mix this compound or compounds with one or more of the metals constituting a comparatively 30 small percentage of the alloy, such as the tungsten, molybdenum, vanadium and others, which are ordinarily alloyed with steel and to add the combination to a molten bath of the other metals.

35 Among the compounds which may be used singly or in combination in the production of alloys according to my invention are silicic acid, titanic acid, vanadic acid, niobic acid and tantalic acid. Boric acid may also 40 be used singly or preferably in combination with any one or more of the first mentioned materials, for the reason that the best results are secured when the added material has a higher fusing point than has the boric 45 acid. The material used in any particular case should be acid with respect to the oxide of at least one of the constituent alloy metals and, preferably with respect to all.

The intimate association of the acid material with one or more of the alloy metals is 50 highly desirable. This may be secured by first precipitating a compound or mixture of tungstic acid, for example, with silicic acid and afterwards reducing to the metal

tungsten impregnated with silica. While 55 this is the preferred method, excellent results may also be obtained by mechanically mixing these materials, as by ball milling.

The results which are obtained through 60 my invention are probably capable of explanation by various theories, both physical and chemical. However, the explanation which seems to be most plausible is that the acid material causes a purification of the 65 metals with which it is associated and this purification takes place just at the time when the alloying takes place. The result is the elimination of oxides and a more perfect 70 union of the constituent alloy metals. The slag formed by the combination of the acid 75 material with these oxides will rise to the surface of the molten bath and may be removed.

A specific example of my invention is the 80 production of a superior quality of high speed steel. In two instances I have added to about 150 parts, by weight, of steel having therein small percentages of chromium and vanadium which are generally used for high speed steel, about 21 parts of a mixture 85 containing substantially 98% tungsten and 2% silica. The silica was incorporated with the tungsten in the manner described in Pacz application, Serial No. 149,915, filed February 20, 1917. This application describes 90 the production of tungsten and at one stage thereof is formed a pressed slug or briquette of finely divided tungsten having silica interspersed therein. Slugs of 95 this kind may be added to the molten steel and there is less chance of oxidation of the tungsten than if an unagglomerated mixture were added. However, good results may be obtained by adding the intimately mixed powder. In another instance I have added 100 to about 150 pounds of steel 21 pounds of a mixture containing 95% tungsten and 5% silica. The products thus derived were given the usual heat treatment, which consists in first annealing, forging down to shape and then hardening the tool by heating to about 1300° C. and quenching quickly in oil or air blast. In both cases the cross section of the steel when broken had an appearance quite different than that of other 105 high speed steels.

I have found that my invention permits the incorporation of a considerably higher

percentage of carbon with the steel than heretofore without destroying the workability thereof. More tungsten may be incorporated with the same percentage carbon.

5. It is to be understood that the intimate mixing of the silica or other acid material with the various metals comprehends not only the chemical method described in the Pacz application hereinbefore referred to 10 but also thorough mechanical mixing.

What I claim is:

1. The method of producing alloys which consists in intimately mixing with one or more of the alloy metals a material which 15 is acid with respect to the oxide of at least one of the alloy metals and adding the combination to a molten bath of the other metal or metals.

2. The method of producing alloys which 20 consists in bringing together under fusing conditions two or more metals, at least one of which is intimately mixed with a material which is acid with respect to the oxide of at least one of these metals.

25. 3. The method of producing alloy steel which consists in adding to a bath of molten steel an alloying metal with which is intimately mixed a material acid with respect to the oxide of said metal.

30. 4. The method of producing alloy steel which consists in adding to a bath of molten steel an alloying metal with which is intimately mixed a material acid with respect to iron oxide.

35. 5. The method of producing alloy steel which consists in adding to a bath of molten steel an alloying metal with which is inti-

mately mixed a material acid with respect to iron oxide and oxide of said metal.

6. The method of producing alloy steel 40 which consists in adding to a bath of molten steel tungsten with which is intimately mixed a material acid with respect thereto.

7. The method of producing alloy steel 45 which consists in adding to a molten steel bath tungsten intimately mixed with silica.

8. The method of producing alloys which consists in adding to a molten bath of one or more metals a briquette containing one or more of the alloy metals intimately mixed 50 with a material acid with respect to the oxide of at least one of the said metals.

9. The method of producing alloy steel which consists in adding to a bath of molten steel a briquette consisting of a metal or 55 ordinarily used in alloy steels intimately mixed with a material acid with respect to the oxide of said metal.

10. The method of producing alloy steel which consists in adding to a bath of molten 60 steel a briquette containing a metal ordinarily used for producing alloy steels and intimately mixed with silica.

11. The method of producing high speed steel which consists in adding to a molten 65 steel bath a briquette containing one or more of the metals ordinarily used to produce high speed steel intimately mixed with silica.

ALADAR PACZ.

Witnesses:

J. H. ANDERSON,  
JOHN E. RYAN,